

1  
2,809,156

## ELECTRODEPOSITION OF IRON AND IRON ALLOYS

William H. Safranek, Columbus, Ohio, assignor, by mesne assignments, to Rockwell Spring & Axle Company, Coraopolis, Pa., a corporation of Pennsylvania

No Drawing. Application August 2, 1954,  
Serial No. 447,403

18 Claims. (Cl. 204—43)

This application relates to electroplating. More specifically, it relates to the electrodeposition of iron and iron-alloy electroplates which are leveling and ductile.

In the process of producing bright, mirrorlike electro-deposits, it has been found necessary to smooth the basis metal surface prior to electrodepositing thereon nickel and chromium plates. This is conventionally done by mechanical finishing operations which consume costly abrasive materials and require the services of skilled operators in order to produce acceptable finishes. The mechanical finishing is done by polishing with a series of finer and finer abrasives which gradually smoothen the rough surfaces in order that a bright, mirrorlike plating can be applied without the necessity of buffing. This is particularly true where very thin coatings of nickel are applied under chromium plating. Unless the surface of the basis material is smooth, the resulting plated finish will not be mirrorlike, but will be hazy or somewhat dull.

It has now been found that by electroplating the leveling iron or iron-alloy coating of this invention on the basis material, a smooth plated surface will be formed, on which extremely thin, bright-nickel, and chromium electroplates can be applied without the necessity for mechanical polishing before plating.

Accordingly, it is one of the objects of this invention to produce an adherent, ductile, leveling iron or iron-alloy electroplate.

It is a further object to produce an adherent electroplate with leveling power suitable as an undercoat for bright-nickel and chromium plates.

Another object is to produce an iron or iron-alloy electroplate which will improve the corrosion resistance of nickel and chromium electroplated thereon.

Other objects and advantageous features will be apparent from the following detailed description.

In general, this invention comprises electrolyzing a bath containing ferrous sulfate, sulfated coconut oxyalcohol, and a leveling agent selected from the group consisting of saccharin and phthalimide. Nickel sulfate and zinc sulfate may be added to produce iron-nickel or iron-nickel-zinc-alloy electroplates. Also, p-toluene sulfonamide may be added to improve both leveling and brightness.

The use of saccharin and p-toluene sulfonamide as brightening agents in acid nickel baths has been disclosed in the patent to Brown, U. S. Patent No. 2,191,813. However, these compounds have been found to have no appreciable leveling action in nickel baths, and it is thus entirely unexpected that when they are used in iron and iron-alloy baths the resulting plate is leveling.

The iron plating bath of this invention comprises an aqueous solution of ferrous sulfate. Very satisfactory results can be obtained using a concentration of from 200 to 600 g./l. of ferrous iron. A preferred amount of ferrous sulfate is from 250 to 400 g./l.

For a satisfactory leveling plate, the ferric ion concentration must not be greater than 0.3 g./l. When the

2

ferric iron concentration does not exceed 0.15 g./l., the plates are more ductile than if this value is exceeded. The ferric ion concentration is reduced by adding iron powder or iron filings, followed by filtration.

5 The organic leveling agent for this bath is selected from the group consisting of saccharin and phthalimide. A preferred amount is from 2 to 3 g./l. Less than 2 g./l. of this organic agent will result in inferior leveling. An amount greater than 3 g./l. may be used, but the resulting plate will have less ductility.

The use of a wetting agent is also necessary to produce leveling plates. Very satisfactory results have been obtained by adding to the bath sulfated coconut oxyalcohol. This is formed by the reaction of coconut alcohol with ethylene oxide, followed by sulfation. The amount of wetting agent used can range from 0.025 to 0.2 g./l.

15 The pH of the bath may be adjusted by adding any suitable material which will not introduce undesirable materials into the bath. Examples of such materials are 20 sulfuric acid for reducing the pH, and iron powder for raising the pH. The pH of the bath should be maintained at from 1.8 to 3.7, although a range of from 2.1 to 2.5 will result in more freedom from pitting and the formation of nodules.

25 During plating, the bath should be maintained at a temperature of from 120° F. to 200° F. However, better leveling is obtained within a range of from 130° F. to 165° F.

It will be obvious to those skilled in the art that the 30 addition of a buffer such as boric acid, may be desirable. Any amount up to saturation may be used in the bath, but from 20 to 45 g./l. is preferred.

Cathode current densities used in producing the plate 35 of this invention may range from 20 to 100 amp./sq. ft. However, the use of current densities ranging from 40 to 75 amp./sq. ft. will produce a more leveling plate and prevent burning at the edges.

Anode current densities up to 50 amp./sq. ft. may be used, although when over 40 amp./sq. ft. is used, the 40 ferric ion concentration may build up.

Agitation during plating may be desirable. This may be accomplished by a moving work bar, a mixer, solution circulation, etc. Filtration of the plating solution may also be desirable to remove insoluble impurities.

45 As has been previously stated, a leveling iron-nickel-alloy plate may be produced by addition of nickel sulfate to the iron sulfate bath. Up to 250 g./l. of nickel sulfate may be added. In addition to the nickel sulfate, up to 10 g./l. zinc sulfate may also be added to the bath to produce an iron-nickel-zinc-alloy electroplate.

The leveling of the baths of this invention may be further improved by the addition of p-toluene sulfonamide in amounts up to 2.0 g./l.

50 The following examples show bath compositions and 55 operating conditions to form the electroplate of this invention on a steel basis material. Iron anodes were used in all of these examples.

## Example 1

|                                          |              |            |
|------------------------------------------|--------------|------------|
| Ferrous sulfate ( $FeSO_4 \cdot 7H_2O$ ) | g./l.        | 300        |
| Saccharin                                | g./l.        | 2.5        |
| Sulfated coconut oxyalcohol              | g./l.        | 0.05       |
| Boric acid ( $H_3BO_4$ )                 | g./l.        | 30         |
| pH                                       |              | 2.1        |
| 60 Temperature                           | °F.          | 160        |
| Cathode current density                  | amp./sq. ft. | 50         |
| Anode current density                    | amp./sq. ft. | 25         |
| Filtration                               |              | Continuous |
| Ferric ion concentration                 | g./l.        | <0.3       |
| Plating time                             | min.         | 25         |
| Leveling                                 | percent      | 50         |

## Example II

|                                                        |              |            |
|--------------------------------------------------------|--------------|------------|
| Ferrous sulfate (FeSO <sub>4</sub> ·7H <sub>2</sub> O) | g./l.        | 300        |
| Saccharin                                              | g./l.        | 2          |
| p-Toluene sulfonamide                                  | g./l.        | 1.75       |
| Sulfated coconut oxyalcohol                            | g./l.        | 0.05       |
| Boric acid (H <sub>3</sub> BO <sub>4</sub> )           | g./l.        | 31         |
| pH                                                     |              | 2.2        |
| Temperature                                            | ° F.         | 160        |
| Cathode current density                                | amp./sq. ft. | 50         |
| Anode current density                                  | amp./sq. ft. | 30         |
| Filtration                                             |              | Continuous |
| Ferric ion concentration, about                        | g./l.        | 0.1        |
| Plating time                                           | min.         | 25         |
| Leveling                                               | percent      | 50         |

## Example III

|                                                        |              |            |
|--------------------------------------------------------|--------------|------------|
| Ferrous sulfate (FeSO <sub>4</sub> ·7H <sub>2</sub> O) | g./l.        | 300        |
| Nickel sulfate                                         | g./l.        | 50         |
| Saccharin                                              | g./l.        | 3          |
| Sulfated coconut oxyalcohol                            | g./l.        | 0.05       |
| pH                                                     |              | 2.3        |
| Temperature                                            | ° F.         | 160        |
| Cathode current density                                | amp./sq. ft. | 50         |
| Anode current density                                  | amp./sq. ft. | 25         |
| Filtration                                             |              | Continuous |
| Ferric ion concentration                               | g./l.        | 0.22       |
| Plating time                                           | min.         | 25         |
| Leveling                                               | percent      | 55-58      |
| Nickel content of plate                                | do           | 3          |

## Example IV

|                                                        |              |       |
|--------------------------------------------------------|--------------|-------|
| Ferrous sulfate (FeSO <sub>4</sub> ·7H <sub>2</sub> O) | g./l.        | 300   |
| Nickel sulfate (NiSO <sub>4</sub> ·6H <sub>2</sub> O)  | g./l.        | 90    |
| Saccharin                                              | g./l.        | 2     |
| Sulfated coconut oxyalcohol                            | g./l.        | 0.05  |
| Boric acid (H <sub>3</sub> BO <sub>4</sub> )           | g./l.        | 30    |
| pH                                                     |              | 2.3   |
| Temperature                                            | ° F.         | 130   |
| Cathode current density                                | amp./sq. ft. | 50    |
| Anode current density                                  | amp./sq. ft. | 25    |
| Ferric ion concentration                               | g./l.        | <0.3  |
| Plating time                                           | min.         | 25    |
| Leveling                                               | percent      | 42-50 |
| Nickel content of plate                                | do           | 15    |

## Example V

|                                                        |              |            |
|--------------------------------------------------------|--------------|------------|
| Ferrous sulfate (FeSO <sub>4</sub> ·7H <sub>2</sub> O) | g./l.        | 300        |
| Nickel sulfate (NiSO <sub>4</sub> ·6H <sub>2</sub> O)  | g./l.        | 250        |
| Saccharin                                              | g./l.        | 2.5        |
| Sulfated coconut oxyalcohol                            | g./l.        | 0.05       |
| pH                                                     |              | 2.3        |
| Temperature                                            | ° F.         | 155        |
| Cathode current density                                | amp./sq. ft. | 50         |
| Anode current density                                  | amp./sq. ft. | 25         |
| Filtration                                             |              | Continuous |
| Ferric ion concentration                               | g./l.        | <0.3       |
| Plating time                                           | min.         | 25         |
| Leveling                                               | percent      | 42-50      |
| Nickel content of plate                                | do           | 15         |

## Example VI

|                                                        |              |      |
|--------------------------------------------------------|--------------|------|
| Ferrous sulfate (FeSO <sub>4</sub> ·7H <sub>2</sub> O) | g./l.        | 300  |
| Nickel sulfate (NiSO <sub>4</sub> ·6H <sub>2</sub> O)  | g./l.        | 90   |
| Saccharin                                              | g./l.        | 2    |
| Sulfated coconut oxyalcohol                            | g./l.        | 0.05 |
| Boric acid (H <sub>3</sub> BO <sub>4</sub> )           | g./l.        | 30   |
| pH                                                     |              | 3.7  |
| Temperature                                            | ° F.         | 160  |
| Cathode current density                                | amp./sq. ft. | 50   |
| Anode current density                                  | amp./sq. ft. | 25   |
| Ferric ion concentration                               | g./l.        | <0.3 |
| Plating time                                           | min.         | 25   |
| Leveling                                               | percent      | 25   |

## Example VII

|                                                        |              |      |
|--------------------------------------------------------|--------------|------|
| Ferrous sulfate (FeSO <sub>4</sub> ·7H <sub>2</sub> O) | g./l.        | 300  |
| Nickel sulfate (NiSO <sub>4</sub> ·6H <sub>2</sub> O)  | g./l.        | 10   |
| Phthalimide                                            | g./l.        | 1    |
| Sulfated coconut oxyalcohol                            | g./l.        | 0.05 |
| Boric acid (H <sub>3</sub> BO <sub>4</sub> )           | g./l.        | 30   |
| pH                                                     |              | 2.3  |
| Temperature                                            | ° F.         | 130  |
| Cathode current density                                | amp./sq. ft. | 50   |
| Anode current density                                  | amp./sq. ft. | 20   |
| Ferric ion concentration                               | g./l.        | <0.3 |
| Plating time                                           | min.         | 25   |
| Leveling                                               | percent      | 50   |

## Example VIII

An electroplate was prepared under the same conditions as Example VII, except that the bath was maintained at a temperature of 160° F. during plating. Comparable results were obtained.

## Example IX

|                                                        |              |            |
|--------------------------------------------------------|--------------|------------|
| Ferrous sulfate (FeSO <sub>4</sub> ·7H <sub>2</sub> O) | g./l.        | 200        |
| Nickel sulfate (NiSO <sub>4</sub> ·6H <sub>2</sub> O)  | g./l.        | 33         |
| Saccharin                                              | g./l.        | 2          |
| p-Toluene sulfonamide                                  | g./l.        | 1.25       |
| Sulfated coconut oxyalcohol                            | g./l.        | 0.05       |
| Boric acid (H <sub>3</sub> BO <sub>4</sub> )           | g./l.        | 20         |
| pH                                                     |              | 2.2        |
| Temperature                                            | ° F.         | 150        |
| Cathode current density                                | amp./sq. ft. | 60         |
| Anode current density                                  | amp./sq. ft. | 30         |
| Filtration                                             |              | Continuous |
| Ferric ion concentration                               | g./l.        | 0.15       |
| Plating time                                           | min.         | 20         |
| Leveling                                               | percent      | Good       |
| Nickel content of plate                                | percent      | 3          |

## Example X

|                                                        |              |                |
|--------------------------------------------------------|--------------|----------------|
| Ferrous sulfate (FeSO <sub>4</sub> ·7H <sub>2</sub> O) | g./l.        | 300            |
| Nickel sulfate (NiSO <sub>4</sub> ·6H <sub>2</sub> O)  | g./l.        | 56             |
| Saccharin                                              | g./l.        | 2              |
| p-Toluene sulfonamide                                  | g./l.        | 1.75           |
| Sulfated coconut oxyalcohol                            | g./l.        | 0.1            |
| Boric acid (H <sub>3</sub> BO <sub>4</sub> )           | g./l.        | 30             |
| pH                                                     |              | 2.1            |
| Temperature                                            | ° F.         | 150            |
| Cathode current density                                | amp./sq. ft. | 90             |
| Anode current density                                  | amp./sq. ft. | 45             |
| Filtration                                             |              | Continuous     |
| Ferric ion concentration                               | g./l.        | <0.2           |
| Plating time                                           | min.         | 20             |
| Leveling                                               | percent      | Good           |
| Nickel content of plate                                | percent      | Not determined |

## Example XI

|                                                        |              |            |
|--------------------------------------------------------|--------------|------------|
| Ferrous sulfate (FeSO <sub>4</sub> ·7H <sub>2</sub> O) | g./l.        | 600        |
| Nickel sulfate (NiSO <sub>4</sub> ·6H <sub>2</sub> O)  | g./l.        | 106        |
| Saccharin                                              | g./l.        | 2          |
| p-Toluene sulfonamide                                  | g./l.        | 1.75       |
| Sulfated coconut oxyalcohol                            | g./l.        | 0.05       |
| Boric acid (H <sub>3</sub> BO <sub>4</sub> )           | g./l.        | 60         |
| pH                                                     |              | 2.2        |
| Temperature                                            | ° F.         | 150        |
| Cathode current density                                | amp./sq. ft. | 60         |
| Anode current density                                  | amp./sq. ft. | 30         |
| Filtration                                             |              | Continuous |
| Ferric ion concentration                               | g./l.        | 0.15       |
| Plating time                                           | min.         | 20         |
| Leveling                                               | percent      | Good       |
| Nickel content of plate                                | percent      | 3          |

## Example XII

|                                                        |              |       |
|--------------------------------------------------------|--------------|-------|
| Ferrous sulfate (FeSO <sub>4</sub> ·7H <sub>2</sub> O) | g./l.        | 300   |
| Nickel sulfate (NiSO <sub>4</sub> ·6H <sub>2</sub> O)  | g./l.        | 90    |
| Zinc sulfate (ZnSO <sub>4</sub> ·7H <sub>2</sub> O)    | g./l.        | 7     |
| Saccharin                                              | g./l.        | 2     |
| Sulfated coconut oxyalcohol                            | g./l.        | 0.05  |
| Boric acid (H <sub>3</sub> BO <sub>4</sub> )           | g./l.        | 30    |
| pH                                                     |              | 2.3   |
| Temperature                                            | °F           | 160   |
| Cathode current density                                | amp./sq. ft. | 50    |
| Anode current density                                  | amp./sq. ft. | 25    |
| Ferric ion concentration                               | g./l.        | <0.3  |
| Plating time                                           | min.         | 25    |
| Leveling                                               | percent      | 40-50 |

The plates produced by all of the foregoing examples were bright, smooth, pit-free, and adherent. As a result of the leveling action, they are capable of being plated further with bright nickel and chromium to produce a brilliant, mirrorlike surface.

It has been further discovered that the plating of this invention results in unusual resistance to corrosion when overplated with nickel and chromium. Steel coated with the plate produced by Example IV (6% nickel) was covered with 0.0001 inch bright nickel and 0.00001 inch chromium. No excessive rusting was noticed after 50 hours of salt-spray testing. When the steel was coated with 0.001 inch of a conventional iron-nickel alloy (15% nickel) and the same amount of nickel and chromium, the steel was protected for only 14 to 40 hours salt-spray testing.

Steel coated with the plating of Example I, plus 0.0003 inch of bright nickel, plus 0.00001 inch of chromium, resisted excessive rusting for 84 hours of salt-spray testing, while the same amount of nickel and chromium protected the steel for only 49 hours.

As can be seen from the foregoing specification, there has been disclosed a novel method for producing a leveling coating of iron and iron alloys wherein the roughness of the basis material can be materially reduced without resorting to mechanical smoothing operations. The quantitative data on leveling given in the above examples refer to the reduction in roughness measured by a diamond point surface analyzer in terms of R. M. S. micro-inches. It has further been disclosed that the iron and iron-alloy plates of this invention afford superior protection against corrosion for the basis material when overplated with nickel and chromium.

What is claimed is:

1. The process of electrodepositing a plating selected from the group consisting of iron and iron base alloys which comprises electrolyzing an aqueous solution containing predominantly ferrous sulfate, a minor amount of an organic compound selected from the group consisting of saccharin and phthalimide and a small quantity of a wetting agent, said amount and quantity being sufficient to provide a level and ductile plate.

2. The process of electrodepositing a plating selected from the group consisting of iron and iron base alloys which comprises electrolyzing an aqueous solution containing predominantly ferrous sulfate, a minor amount of an organic compound selected from the group consisting of saccharin and phthalimide, and a small quantity of sulfated coconut oxyalcohol, said amount and quantity being sufficient to provide a level and ductile plate.

3. The process of electrodepositing a plating selected from the group consisting of iron and iron base alloys which comprises electrolyzing an aqueous solution containing predominantly ferrous sulfate, 2 to 3 g./l. of an organic compound selected from the group consisting of

70

50

45

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

## 6

saccharin and phthalimide, and 0.025 to 0.2 g./l. of sulfated coconut oxyalcohol.

4. A composition of matter for electrodepositing a plating selected from the group consisting of iron and iron base alloys which comprises an aqueous solution containing predominantly ferrous sulfate, a minor amount of an organic compound selected from the group consisting of saccharin and phthalimide, and a small quantity of a wetting agent, said amount and quantity being sufficient to provide a level and ductile plate.

5. A composition of matter for electrodepositing a plating selected from the group consisting of iron and iron base alloys which comprises an aqueous solution containing predominantly ferrous sulfate, a minor amount of an organic compound selected from the group consisting of saccharin and phthalimide, and a small quantity of sulfated coconut oxyalcohol, said amount and quantity being sufficient to provide a level and ductile plate.

6. A composition of matter for electrodepositing a plating selected from the group consisting of iron and iron base alloys which comprises an aqueous solution containing predominantly ferrous sulfate, 2 to 3 g./l. of an organic compound selected from the group consisting of saccharin and phthalimide, and 0.025 to 0.2 g./l. of sulfated coconut oxyalcohol.

7. The process of electrodepositing a plating selected from the group consisting of iron and iron base alloys which comprises electrolyzing an aqueous solution containing from 250 to 400 g./l. of ferrous sulfate, 2 to 3 g./l. of an organic compound selected from the group consisting of saccharin and phthalimide, and 0.025 to 0.2 g./l. of sulfated coconut oxyalcohol.

8. A composition of matter for electrodepositing a plating selected from the group consisting of iron and iron base alloys which comprises an aqueous solution containing from 250 to 400 g./l. of ferrous sulfate, 2 to 3 g./l. of an organic compound selected from the group consisting of saccharin and phthalimide, and 0.025 to 0.2 g./l. of sulfated coconut oxyalcohol.

9. The process according to claim 2 wherein the aqueous solution additionally contains nickel sulfate.

10. The process according to claim 9 wherein the aqueous solution additionally contains zinc sulfate.

11. The process according to claim 2 wherein the aqueous solution additionally contains p-toluenesulfonamide.

12. The process according to claim 9 wherein the aqueous solution additionally contains p-toluenesulfonamide.

13. The process according to claim 10 wherein the aqueous solution additionally contains p-toluenesulfonamide.

14. The composition according to claim 5 containing additionally nickel sulfate.

15. The composition according to claim 14 containing additionally zinc sulfate.

16. The composition according to claim 5 containing additionally p-toluenesulfonamide.

17. The composition according to claim 14 containing additionally p-toluenesulfonamide.

18. The composition according to claim 15 containing additionally p-toluenesulfonamide.

## References Cited in the file of this patent

## UNITED STATES PATENTS

1,072,091 Cowper-Coles Sept. 2, 1913  
2,420,403 Stoddard May 13, 1947

## FOREIGN PATENTS

525,847 Great Britain Sept. 5, 1940  
589,561 Great Britain June 24, 1947  
614,038 Great Britain Dec. 8, 1948